# NEW EUROPEAN PATENT SPECIFICATION

(11) **EP 0 136 727 B2**
(45) Date of publication and mention of the opposition decision: **07.10.1992**
(45) Mention of the grant of the patent: 12.08.1987
(21) Application number: 84200913.6
(22) Date of filing: 25.06.1984
(51) Int. Cl.: D06M 15/244, D02G 1/16, F16J 15/22

(54) **Aromatic polyamide yarn impregnated with lubricating particles, a process for the manufacture of such a yarn, and packing material or rope containing this yarn**
Mit schmierenden Partikeln imprägniertes aromatisches Polyamidgarn, Verfahren zur Herstellung dieses Garnes und dasselbe enthaltendes Dichtungsmaterial oder Seil
Fil en polyamide aromatique imprégné de particules lubrifiantes, procédé pour sa fabrication et matériau de garniture ou corde contenant ce fil

(30) Priority: 04.07.1983 NL 8302368
(43) Date of publication of application: 10.04.1985
(73) Proprietor: AKZO N.V., NL-6824 BM Arnhem (NL)
(72) Inventor: van Anholt, Willem Carel, NL-6823 JK Arnhem (NL); Peters, Martinus Wilhelmus M. G., NL-6521 KK Nijmegen (NL)
(74) Representative: Miggelenbrink, Evert Willem

(56) References cited:
- DE-A- 2 326 826
- US-A- 2 807 864
- US-A- 3 110 151
- US-A- 3 302 386
- US-A- 3 306 155
- US-A- 3 827 114
- US-A- 4 232 087
- US-A- 4 371 180

## Description

The invention relates to a yarn comprising aromatic polyamides, which yarn is impregnated with a dispersion containing solid, lubricating particles, particularly particles of polytetrafluoroethylene.

The invention also comprises a process for the manufacture of such yarn, and packing material, for instance stuffing box packing, consisting of said yarn.

A yarn of the type indicated above is known from US-A-4 371 180, which describes packing composed of braided inorganic yarns, preferably of glass, and of braided organic yarns, preferably of polytetrafluoroethylene or wholly aromatic polyamides. Before or after being braided, the yarn may be impregnated with a dispersion of solid particles of a fluorine-containing polymer and starch. The dispersion containing polytetrafluoroethylene (PTFE) particles contributes considerably to the sealing properties of the end product in the form of packing material. Although the results obtained with the packing material disclosed in US-A-4 371 180 are reasonable, the present invention makes it possible to improve on these results. It should be added that DE-A-23 26 826 describes a blended yarn consisting of 50-80% by weight of PTFE filaments and 50-20% by weight of aromatic polyamide filaments. Said blended yarn is coated with fine PTFE particles and may in the braided form be used as packing material. Before these two yarns are coated with PTFE particles, they must be assembled, which may optionally be effected by the blowing process described in US-A-3 110 151. This blowing process results in a smooth yarn free of loops and therefore not bulky or textured. Coating such a yarn with PTFE particles will consequently result in these particles being practically entirely present on the outside of the yarn. Further, considering that the yarn according to DE-A-23 26 826 is a blend of two yarns having widely different properties, it is less homogeneous than a yarn of one and the same material.

Reference is also made to EP-A-0 032 744, which discloses a wholly aromatic polyamide yarn provided with a fluoro compounds-containing polymer. In that case the fluoro compound is not present on the fibres in the form of separate particles, but in the form of a continuous coating. As the PTFE is not present then on the fibres in the form of separate particles, this known yarn is not suitable to be used as packing yarn.

Further reference is made to CA-A 995 288 describing a hovercraft skirt containing an elastomer coated fabric composed of looped yarn textured by air under pressure, which yarns preferably consist of wholly aromatic polyamides. Therefore, looped yarns of aramids textured under air pressure are known in themselves from CA-A-995 288, but their field of appliation is entirely different and they are not at all meant to be used in combination with PTFE particles.

According to the present invention an improved yarn from wholly aromatic polyamide has been developed in the first place for use in packing material. The yarn according to the invention consists of aromatic polyamide endless filaments which are impregnated with a dispersion containing solid lubricating particles of polyfluorocarbon resins, more particularly PTFE, and/or graphite, wherein the yarn is a tangled loopy yarn interlaced with an overfeed of at least 1 % by a fluid-jet process. According to the invention the solid particles may consist of a polyfluorocarbon resin, more particularly polytetrafluoroethylene, or of graphite. Alternatively, however, use may be made of a mixture of solid particles of a polyfluorocarbon resin and of graphite. The wet yarn subjected to a fluid-jet treatment according to the invention has a voluminous character, which renders the yarn according to the invention particularly suitable for taking up a lubricant. Owing to its voluminous character the yarn will readily absorb a large amount of lubricant, which makes the yarn according to the invention particularly suitable to be formed into a packing material. As lubricants commonly used in the packing industry for impregnating yarns may be mentioned: paraffin oil, silicone oil or molybdenum disulphide or some other suitable lubricant, depending on the field of application of the packing to be manufactured. The invention comprises in particular a yarn which is so voluminous that the absorption capacity for a lubricant of the polyfluorocarbon particles-containing yarn is in the range of 20 to 50 per cent by weight, preferably in the order of 35 per cent by weight, calculated on the weight of the dry yarn provided with solid PTFE and/or graphite particles. The lubricant contributes considerably to the gas and/or liquid tightness and the frictional behaviour of a packing material. After being successively impregnated with PTFE particles, braided to form a packing material, and impregnated with a lubricating agent the aramid yarn according to the invention is capable of ensuring a long service life as far as high gas and/or liquid tightness and lubricating effect are concerned. According to the invention the yarn contains 1000 to 20 000 filaments, preferably about 5000 filaments, and the linear density of the yarn is in the range of tex 150 to 3000, preferably in the order of tex 850. According to the invention the yarn need contain only a relatively small proportion of solid PTFE and/or graphite particles, namely less than 60 per cent by weight, preferably 10-45% by weight, and more particularly about 20% by weight, calculated on the dry weight of the yarn without the solid particles. According to the invention the size of 80% of the solid particles is preferably in the range of about 0,1 to 1 f,.lm. The yarn according to the invention is particularly characterized in that the solid particles are so evenly applied to the yarn that measured in a random cross-section of the yarn at least 50%, preferably 70% to 100% of the number of filaments are provided with one or more of said particles.

The special configuration of the yarn due to the wet-blowing process permits a particular uniform distribution of the PTFE particles over the cross-sectional area of the yarn. As a result, the function of the PTFE particles present in the yarn, i.e. promoting the sealing action of the packing material, is rendered most effective. Moreover, the PTFE particles enhance the chemical resistance of the packing material and reduce friction. The yarn according to the invention can therefore be formed into a packing material which ensures sufficient sealing over a long service time even under high dynamic loads, as in the case of high speed shafts or reciprocating parts in combination with elevated temperature and pressure and, possibly, a chemically agressive medium. Further, as a result of the uniform distribution of the PTFE particles over practically all the filaments of the yarn only a relatively small amount of PTFE particles is needed for this yarn of the present invention to be made into a satisfactorily sealing packing material. Another advantage of the uniform distribution of the PTFE particles in the yarn according to the invention consists in that the packing into which the yarn is braided need not be additionally impregnated with a PTFE particles-containing dispersion.

The yarn according to the invention has been especially developed and made suitable to be worked up into a packing material, such as stuffing box packing, which is widely used in machine construction for the sealing of rotating shafts and reciprocating parts. In the manufacture of packing material a number of yarns of the invention impregnated with PTFE and/or graphite particles can be braided together on a packing braiding machine to form a packing material which may for instance have a rectangular cross-section. The braided packing material is generally impregnated with a lubricating agent. such as a special oil, fat or other substances required in view of the use of the packing material. In the completed packing material according to the invention the proportion by weight of solid particles, calculated on the dry weight of the aramid yarn without solid particles, may be lower than 60%, and is preferably 10 to 45%. The invention particularly comprises a packing material of aromatic polyamide yarn impregnated with solid PTFE and/or graphite particles, which packing material is characterized in that it contains a fairly large amount of said lubricating agent, viz. an amount of 20 to 50% by weight, preferably about 25% by weight, calculated on the weight of the dry yarn provided with solid particles.

A simple and effective method of manufacturing the yarn according to the invention comprises the application to the yarn of a dispersion of solid particles of polyfluorocarbon resins and/or graphite. Whilst in the wet state the yarn is subjected to a blowing process using a fluid under pressure, more particularly air, as a result of which the solid particles are distributed over the filaments and the filaments are generally interentangled and braided. According to a preferred embodiment of the process according to the invention the yarn is subjected to a blowing process after the dispersion of solid particles of a polyfluorocarbon resin-containing and/or graphite particles-containing dispersion has been applied to the yarn. Alternatively, according to the invention, the. dispersion of particles of a polyfluorocarbon resin and/ or graphite may be directly blown onto the yarn while being fed to it under pressure. In the blowing process air is used at an absolute pressure of 3 to 10 bar.

According to a preferred embodiment of the process of the present invention the, preferably positively charged, PTFE are applied to the yarn from an aqueous dispersion whose composition may substantially be as follows:
45 to 75% by weight of PTFE particles, preferably about 58% by weight;
50 to 20% by weight of water, preferably about 40% by weight;
not more than 5% by weight of a wetting agent based on alkylphenoxyethanol, preferably about 3,5% by weight.

The graphite particles are also applied from an aqueous dispersion, which may contain, for instance, about 18% by weight of graphite and 82% by weight of water and a nonionic wetting agent.

Particularly favourable results may be obtained when the PTFE and/or graphite particles are applied to the yarn from said dispersion with the aid of a kiss roll. Optionally, the PTFE and/or graphite particles may be applied to the yarn by passing it through a bath of said dispersion.

According to the invention the yarn is fed to the blowing process at a rate in excess of that at which it is withdrawn therefrom of at least 1 %, preferably about 3% to 6%.

Furthermore, the yarn according to the invention is particularly suitable to be used in the manufacture of rope having an outer diameter of, for example 3 to 100 mm such as marine rope, hoisting rope and the like, which rope is built up of two or more strands by laying or braiding. According to the invention the yarn to be incorporated in such rope contains less than 10% by weight, preferably about 5% by weight of solid particles.

The invention will be illustrated with reference to the accompanying schematic drawing.
Figure 1 shows an apparatus for applying PTFE particles to the yarn before the blowing process.
Fig. 2 shows a somewhat modified apparatus for carrying out the process of the invention.

In the embodiment shown in Figure 1 the process is started from 5 packages 1 of non-twisted aramid filament yarn. The aramid yarn 2 of each of the packages has 1000 filaments and a linear density of tex 168 and contains about 0,8% of a finish applied to the yarn during spinning. The five aramid filament yarns 2 are assembled by the schematically indicated yarn guide 3 and drawn off from the starting packages 1 by the driven rolls 4,5. The assembled yarn 6 is subsequently run over the kissing roll 7 rotating in an aqueous dispersion 8. The assembled filament yarn thus wetted and provided with PTFE and/or graphite particles is fed to a blow box 9 containing an air nozzle 10 at a rate in excess of the rate at which it is withdrawn from the blow box. The nozzle 10 may be of the type as indicated in US-A-3 302 386. The blown and impregnated yarn is discharged from the blow box 9 over a pair of driven pulling-off rolls 11,12 which have such a lower circumferential speed than the feed rolls 4,5 as to ensure that the yarn is fed to the air nozzle 10 at a sufficiently high excess feed rate. After leaving the heated pulling-off rolls 11,12 the dried yarn may still be lubricated, if desired, and subsequently wound into a package.

In the blow box 9 the assembled yarn 5x168 composed of 5 basic yarns 2 is treated with air at an absolute pressure of 5 bar, the yarn being fed at an excess rate of 3%. Alternatively, the asembled yarn may be made up of 10 basic yarns. Such assembled 10x168 tex yarn is treated in the blow box 9 with air fed at an absolute pressure of 10 bar, the excess feed rate of the yarn being 6%. When the yarn is treated without applying an excess feed rate, it may be fed to and discharged from the blowing zone at a speed of 60 min/ min.

Fig. 2 shows a somewhat modified embodiment of the apparatus for carrying out the process according to the invention. The untreated aramid yarn 13 is fed by a pair of rolls 14 at a particular speed desired. After leaving the rolls 14 the yarn is passed through a bath 15 containing an aqueous dispersion of PTFE and/or graphite particles. In the bath the yarn is passed over two or more guide rolls (not shown in the drawing). After leaving the bath 15 the yarn passes upwards through a feed pipe 17 ending in a blow box 18. In the blow box 18 there is again a nozzle (not shown) of the type described in US-A-3 302 386. The advantage of the feed pipe 17 is that excess dispersion not entrained by the yarn and blown off from the yarn flows back into the bath through said pipe 17. After having been subjected to the blowing treatment, the impregnated yarn 19 leaves the blow box 18 through the outlet opening 20. The yarn is withdrawn from the blow box 18 by the driven roll 24 with separator roll 21. The roll 24 may be heated for drying the yarn. The yarn thus impregnated and dried may be formed into a package via a traverse mechanism 22. The circumferential speed of the roll 24 is lower than that of the rolls 14, so that the yarn is passed through the blow box at the particular excess feed rate desired.

It has been found that with the process given in Figure 1 favourable results may be obtained, i.e., viewed in cross-section of the yarn the PTFE particles are very uniformly distributed over practically all the filaments mainly under the following process conditions:
circumferential speed of the kissing roll: 42 m/min;
circumferential speed of the rolls 4,5: 59,5 m/min (yarn feed rate);
circumferential speed of the rolls 11,12: 58 m/min (yarn discharge rate); absolute pressure of the blow air: 3 to 4 bar;
composition of dispersion: 56,5% by weight of PTFE particles, 40% by weight of water and 3,5% by weight of wetting agent of the Triton@ X 100 type, which is a commercially available wetting agent based on alkylphenoxy ethanol.

The dispersion used is of the type marketed by ICI under the name Fluon®; the PTFE particles in it carry a negative electric charge. In the process of the invention, however, also other dispersions may be applied. Use may advantageously be made of dispersions in which the particles of the fluorocarbon compound, more particularly polytetrafluoroethylene (PTFE), carry a positive electric charge. These last-mentioned dispersions are elaborately described in DE-A-26 44152. Use of a dispersion containing positively charged PTFE particles is expected to lead to an even better adhesion of these particles to the filaments of the yarn.

It should be added that the excess feed rate used in the wet-blowing process of the present invention is of great influence on the structure of the yarn. Particularly the interentanglement or interlacement of the filaments is very much dependent on the excess feed rate. At an the excess feed rate of as low as 1 % the non-twisted yarn loses its smooth appearance and becomes somewhat bulky or textured as a result of the interentanglement and/or interlacement of the filaments and the formation of loops in one or more filaments. The interentanglement and interlacement of the filaments of a yarn and the manufacture of a yarn having a multitude of loops are known in themselves from the textile art and are described in US-A-3 302 386 and US-A-2 783 609. The interentanglement and interlacement of the filaments of a yarn with the aid of a blowing process and using an excess feed rate of the yarn imparts a voluminous character to the yarn. A high excess feed rate renders the yarn very bulky. The yarn wetted with a PTFE and/or graphite dispersion and subjected to a blowing treatment has a voluminous character, which is influenced by the degree of impregnation with solid particles. Impregnation of the yarn with a higher percentage of PTFE particles is attended with a lower voluminous character as a result of the adhesion of the PTFE particles to the yarn; in other words, the degree of impregnation to be chosen depends on the voluminous character desired.

In the manufacture of the yarn according to the invention the preferred excess feed rate is in the range of 3% to 6%, which results in a yarn having a more or less loopy character. The presence of internal and/or external loops formed in one or more filaments of the yarn and the resulting bulky appearance is characteristic of a particular embodiment of the yarn according to the invention. Particularly surprising is that already a fairly low excess feed rate of 3% results in a sufficiently voluminous yarn which is excellently suitable to be further processed into a packing material. The blowing process constitutes an essential element of the invention with a view to obtaining a very good distribution of the solid particles over the filaments of the yarn.

Also a smooth, non-air blown aramid filament yarn can be treated with a PTFE particles-containing dispersion, use being made of an applicator roll or impregnation. Experiments, however, have demonstrated that in that case the PTFE particles will stick to the outer circumference of the yarn in the form of variously sized lumps, as can be seen on a highly enlarged photograph of a cross-section of the yarn. Such a photograph also shows that hardly any PTFE particles at all are stuck to the filaments that are within the circumference of the yarn. Therefore, a non-air treated aramid filament yarn cannot be evenly impregnated with PTFE particles and is less suitable to be worked up into a packing material.

The afore-mentioned absorption capacity of the yarn mentioned hereinbefore with regard to lubricants, such a paraffin oil, silicone oil, molybdenum disulphide or the like is referred to as oil absorption capacity and is determined as follows: An one metre long piece of aramid filament yarn impregnated beforehand with PTFE particles is impregnated with paraffin oil having a viscosity of 72 centipoises (72 mPas; measured by the Brook- field method) by dipping the yarn in a tray with paraffin oil at room temperature, after which the tray is kept in a vacuum chamber for 15 minutes. The yarn thus impregnated is suspended by its one end in such a way that the paraffin oil which cannot be retained by the yarn can drip off at its other free end. The amount of paraffin oil absorbed, which is a measure of said oil absorption capacity, is determined by weighing. The second weighing of the oil-impregnated yarn is carried out as soon as there can no longer be observed any dripping at the free end of the yarn after at least 24 hours. To determine the oil absorption capacity the first weighing is carried out on said 1 m long piece of yarn while still dry and impregnated with PTFE and/or graphite particles.

Assume the result of the first weighing to be A units of weight (= dry yarn + PTFE and/or graphite particles).

Assume the result of the second weighing to be B units of weight (= dry yarn + PTFE and/or graphite particles + paraffin oil). The oil absorption capacity C envisaged in accordance with the invention can be calculated then from the formula

If the results A and B of the first and the second weighings are, for instance, 1000 and 1350 weight units, respectively, then

It should be added that by dry aromatic polyamide yarn mentioned in various places in the description is to be understood an aramid yarn which is dried at 100°C to a moisture content of 6% by weight. Said moisture content is defined at 20°C and 65% relative humidity.

The term wholly aromatic polyamides as used with regard to the present invention refers to polyamides which are entirely or substantially built up of recurrent units of the general formula wherein A_{1'} A₂ and A3 represent different or the same divalent, one or more aromatic rings-containing rigid radicals which may also contain a heterocyclic ring, of which radicals the chain extending bonds are in the position para to each other or are parallel and oppositely directed. Examples of these radicals include 1,4-phenylene, 4,4'-biphenylene, 1,5-naphthylene and 2,6-naphthylene.

They may contain substituents or not, e.g. halogen atoms or alkyl groups.

As regards the composition of the aramids it should be added that they may optionally contain up to 35 mole % of other groups, such as m-phenylene groups, non-rigid groups, such as alkyl groups, or ether groups, urea groups or ester groups. As examples of aramids may be mentioned poly-p-benzamide, poly-p-phenylene terephthalamide and their copolymers. According to the invention it is preferred that use should be made of yarns of poly-p-phenylene terephthalamide (PPDT).

Of the fluorine-containing compounds that may advantageously be used for the yarn according to the invention may be mentioned: polytetrafluoroethylene (PTFE), polyhexafluoropropylene, polychlorotrifluoroe- thene, polyvinylidene fluoride, tetrafluoroethene hexafluoropropylene copolymer, vinylidene fluoride-hexafluoropropylene copolymer, fluorosilicone elastomers, polyfluoroaniline, tetrafluoroethene trifluoronitrosomethane copolymer, graphite fluoride, etc.

## Claims

1. A yarn consisting of aromatic polyamide endless filaments which are impregnated with a dispersion containing solid lubricating particles of polyfluorocarbon resins, particularly PTFE, and/or graphite, wherein the yarn is a tangled loopy yarn interlaced with an overfeed of at least 1% by a fluid-jet process.

2. A yarn according to claim 1, characterized in that the yarn is so structured that the absorption capacity for a lubricant of the solid particles-containing yarn is in the range of 20 to 50 percent by weight, preferably in the order of 35 per cent by weight, calculated on the weight of the dry yarn provided with solid particles.

3. Ayarn according to claim 1, characterized in that it has a great many loops formed in one or more filaments.

4. A yarn according to one or more of the preceding claims, characterized in that the yarn contains 1000 to 20 000 filaments, preferably about 5000 filaments, and the linear density of the yarn is in the range of tex 150 to 3000, preferably in the order of tex 850.

5. A yarn according to claim 1, characterized in that the yarn contains less than 60 per cent by weight of solid particles, calculated on the weight of the dry yarn without solid particles.

6. A yarn according to one or more of the preceding claims, characterized in that the solid particles are so evenly applied to the yarn that measured in a random cross-section of the yarn at least 50%, preferably 70% to 100% of the number of filaments are provided with one or more of said particles.

7. A yarn according to one or more of the Preceding claims, characterized in that the size of 80% of the solid particles is less than 1 f,.lm.

8. A yarn according to claim 5, characterized in that the yarn contains 10-45 per cent by weight, preferably about 30% by weight, of solid particles, calculated on the dry weight of the yarn without solid particles.

9. A yarn according to claim 5, characterized in that the yarn contains less than 10 per cent by weight, preferably about 5 per cent by weight, of solid particles, calculated on the dry weight of the yarn without solid particles.

10. A packing material, such as stuffing box packing, characterized in that it consists of the yarn according to one or more of the claims 1-8.

11. A packing material according to claim 10, characterized in that the proportion by weight of the solid particles is smaller than 60%, preferably 10 to 45%, calculated on the weight of the dry yarn without solid particles.

12. A packing material according to claims 10 and 11, characterized in that it contains a lubricating agent, such as paraffin oil, silicone oil, molybdenum disulphide or the like in an amount of 20 to 50 per cent by weight, preferably about 35% by weight, calculated on the weight of the dry yarn of aromatic polyamides provided with solid particles.

13. Rope such as marine rope, hoisting rope and the like, which rope is built up of two or more strands by laying or braiding, characterized in that the rope is formed of the yarn according to claim 9.

14. A process for the manufacture of the yarn according to one or more of the claims 1-9, comprising the application to the yarn of a dispersion of solid lubricating particles of polyfluorocarbon resins, particularly PTFE, and/or graphite, the yarn whilst in the wet state being subjected to an interlacing process using a fluid under pressure, preferably air, as a result of which the solid particles are distributed over the filaments.

15. A process according to claim 14, characterized in that the fluid is blown onto the yarn substantially transverse to the direction of movement thereof.

16. A process according to claim 14, characterized in that the yarn is subjected to a blowing treatment after the application to it of the dispersion containing the solid particles.

17. A process according to claim 14 or 15, characterized in that the solid particles-containing dispersion is applied to the yarn during the blowing process.

18. A process according to claim 17, characterized in that the solid particles-containing dispersion is directly applied to the filaments of the yarn by being blown onto it under pressure.

19. A process according to claim 14, characterized in that negatively charged solid particles of a polyfluorocarbon resin are applied to the yarn-from an aqueous dispersion.

20. A process according to claim 14, characterized in that positively charged particles of a polyfluorocarbon resin are applied to the yarn from an aqueous dispersion.

21. A process according to claim 19 or 20, characterized in that the composition of the aqueous dispersion is substantially as follows:
- 45 to 75% by weight of PTFE particles, preferably about 58% by weight;
- 50 to 20% by weight of water, preferably about 40% by weight;
- nor more than 5% by weight of a wetting agent based on alkylphenoxyethanol, preferably about 3,5% by weight.

22. A process according to claim 14, characterized in that the excess feed rate is at least 1 %, preferably about 3% to 6%.

## Patentansprüche

1. Garn aus aromatischen Polyamid-Endlosfilamenten, die mit einer Dispersion imprägniert sind, welche feste schmierende Partikel aus Polyfluorkohlenstoffharzen, insbesondere PTFE, und/oder Graphit enthält, wobei das Garn ein Schlingen aufweisendes Wirrgarn ist, das mit einem Einspeisungsüberschuss von mindestens 1% durch Fluidstrahlbehandlung verflochten ist.

2. Garn nach Anspruch 1, dadurch gekennzeichnet, dass das Garn so strukturiert ist, dass die Absorptionskapazität des die festen Partikel enthaltenden Garns für ein Schmiermittel im Bereich von 20 bis 50 Gew.%, vorzugsweise in der Grössenordnung von 35 Gew.%, berechnet auf das Gewicht des mit den festen Partikeln versehenen trockenen Garns, liegt.

3. Garn nach Anspruch 1, dadurch gekennzeichnet, dass es viele, in einem Filament oder in mehreren Filamenten gebildete Schlingen aufweist.

4. Garn nach einem oder mehreren dervorangehenden Ansprüche, dadurch gekennzeichnet, dass das Garn 1000 bis 20'000 Filamente, vorzugsweise etwa 5000 Filamente, enthält und der Titer des Garns im Bereich von tex 150 bis 3000, vorzugsweise in der Grössenordnung von tex 850, liegt.

5. Garn nach Anspruch 1, dadurch gekennzeichnet, dass das Garn weniger als 60 Gew.% feste Partikel, berechnet auf das Gewicht des trockenen Garns ohne die festen Partikel, enthält.

6. Garn nach einem oder mehreren der vorangehenden Ansprüche, dadurch gekennzeichnet, dass die festen Partikel derart gleichmässig auf das Garn appliziert sind, dass an einem statistischen Garnquerschnitt mindestens 50%, vorzugsweise 70 bis 100%, der Anzahl der Filamente ein oder mehrere Partikel tragen.

7. Garn nach einem oder mehreren der vorangehenden Ansprüche, dadurch gekennzeichnet, dass 80% der festen Partikel einen Grösse von unter 1f,.lm haben.

8. Garn nach Anspruch 5, dadurch gekennzeichnet, dass das Garn 10 bis 45 Gew.%, vorzugsweise etwa 30 Gew.%, feste Partikel, berechnet auf das Trockengewicht des Garns ohne die festen Partikel, enthält.

9. Garn nach Anspruch 5, dadurch gekennzeichnet, dass das Garn weniger als 10 Gew.%, vorzugsweise etwa 5 Gew.%, feste Partikel, berechnet auf das Trockengewicht des Garns ohne die festen Partikel, enthält.

10. Dichtungsmaterial, z.B. für Stopfbuchsenpackungen, dadurch gekennzeichnet, dass es aus Garn gemäss einem oder mehreren der Ansprüche 1 bis 8 besteht.

11. Dichtungsmaterial nach Anspruch 10, dadurch gekennzeichnet, dass der Gewichtsanteil der festen Partikel kleiner als 60% ist, vorzugsweise 10 bis 45% beträgt, berechnet auf das Gewicht des trockenen Gams ohne die festen Partikel.

12. Dichtungsmaterial nach den Ansprüchen 10 und 11, dadurch gekennzeichnet, dass es ein Schmiermittel, wie Paraffinöl, Siliconöl, Molybdänsulfid oder dgl., in einem Anteil von 20 bis 50 Gew.%, vorzugsweise etwa 35 Gew.%, enthält, berechnet auf das Gewicht des mit den festen Partikeln versehenen trockenen Garns aus aromatischen Polyamiden.

13. Seil, z.B. Schiffsseil, Zugseil oder dgl., das durch Verseilen, Zusammendrehen oder Verflechten von zwei oder mehr Strängen aufgebaut ist, dadurch gekennzeichnet, dass das Seil aus Garn gemäss Anspruch 9 gebildet ist.

14. Verfahren zur Herstellung des Garns nach einem oder mehreren der Ansprüche 1 bis 9 durch Auftragen einer Dispersion von festen schmierenden Partikeln aus Polyfluorkohlenstoffharzen, insbesondere PTFE, und/oder Graphit, auf das Garn, wobei das in nassem Zustand befindliche Garn unter Verwendung eines Fluids, vorzugsweise Luft, unter Druck einer Verschlingungsbehandlung ausgesetzt wird, wodurch die festen Partikel auf den Filamenten verteilt werden.

15. Verfahren nach Anspruch 14, dadurch gekennzeichnet, dass das Fluid praktisch quer zur Bewegungsrichtung des Garns auf dieses geblasen wird.

16. Verfahren nach Anspruch 14, dadurch gekennzeichnet, dass das Garn nach der Applikation der Dispersion, welche die festen Partikel enthält, einem Blasprozess unterzogen wird.

17. Verfahren nach Anspruch 14 oder 15, dadurch gekennzeichnet, dass die Dispersion, welche die festen Partikel enthält, während des Blasprozesses auf das Garn aufgetragen wird.

18. Verfahren nach Anspruch 17, dadurch gekennzeichnet, dass die Dispersion, welche die festen Partikel enthält, direkt durch Aufblasen unter Druck auf die Filamente des Garns aufgebracht wird.

19. Verfahren nach Anspruch 14, dadurch gekennzeichnet, das negativ geladene, feste Polyfluorkohlenstoffharzpartikel aus wässriger Dispersion auf das Garn aufgetragen werden.

20. Verfahren nach Anspruch 14, dadurch gekennzeichnet, dass positiv geladene Polyfluorkohlenstoffharzpartikel aus wässriger Dispersion auf das Garn aufgetragen werden.

21. Verfahren nach Anspruch 19 oder 20, dadurch gekennzeichnet, dass die wässrige Dispersion im wesentlichen folgende Zusammensetzung hat:
45 bis 75 Gew.%, vorzugsweise etwa 58 Gew.%, PTFE-Partikel;
50 bis 20 Gew.%, vorzugsweise etwa 40 Gew.%, Wasser;
höchstens 5 Gew.%, vorzugsweise etwa 3,5 Gew.%, Netzmittel auf Basis von Alkylphenoxyethanol.

22. Verfahren nach Anspruch 14, dadurch gekennzeichnet, dass die Einspeisungsrate mindestens um 1%, vorzugsweise um etwa 3 bis 6%, grösser als die Abführungsrate ist.

## Revendications

1.- Fil constitué de filaments sans fin en polyamide aromatique qui sont imprégnés d'une dispersion contenant des particules lubrifiantes solides de résines polyfluorocarbonées, en particulier de PTFE, et/ou de graphite, dans lequel le fil est un fil en forme de boucle, enchevêtré, entrelacé, avec une suralimentation du fil d'au moins 1% par un procédé à jet de fluide.

2.- Fil selon la revendication 1, caractérisé en ce que le fil est structuré de manière que la capacité d'absorption d'un lubrifiant par le fil contenant les particules solides soit dans l'intervalle de 20 à 50% en poids, de préférence de l'ordre de 35% en poids, calculée par rapport du fil sec comportant les particules solides.

3.- Fil selon la revendication 1, caractérisé en ce qu'il comporte de très nombreuses boucles formées dans un ou plusieurs filaments.

4.- Fil selon l'une quelconque des revendications précédentes, caractérisé en ce que le fil contient 1 000 à 20 000 filaments, de préférence environ 5 000 filaments, et en ce que la masse linéique du fil est dans l'intervalle de 150 à 3 000 tex, de préférence de l'ordre de 850 tex.

5.- Fil selon la revendication 1, caractérisé en ce que le fil contient moins de 60% en poids de particules solides, calculé par rapport au poids du fil sec sans les particules solides.

6.- Fil selon l'une quelconque des revendications précédentes, caractérisé en ce que les particules solides sont appliquées si uniformément au fil que, si on les mesure dans une section droite quelconque du fil, au moins 50%, de préférence 70% à 100%, du nombre des filaments comporte une ou plusieurs desdites particules.

7.- Fil selon l'une quelconque des revendications précédentes, caractérisé en ce que la granulométrie de 80% des particules solide est inférieure à 1 f,.lm.

8.- Fil selon la revendication 5, caractérisé en ce que le fil contient 10-45% en poids, de préférence environ 30% en poids, de particules solides, calculé par rapport au poids sec du fil sans les particules solides.

9.- Fil selon la revendication 5, caractérisé en ce que le fil contient moins de 10% en poids, de préférence environ 5% en poids, de particules solides, calculé par rapport au poids sec du fil sans les particules solides.

10.- Matériau de garniture, comme une garniture de presse-étoupe, caractérisé en ce qu'il consiste en fil selon l'une quelconque des revendications 1 à 8.

11.- Matériau de garniture selon la revendication 10, caractérisé en ce que la proportion en poids des particules solides est inférieure à 60%, de préférence de 10 à 45%, calculée par rapport au poids du fil sec sans les particules solides.

12.- Matériau de garniture selon les revendications 10 et il, caractérisé en ce qu'il contient un agent lubrifiant, comme de l'huile de paraffine, de l'huile de silicone, du bisulfure de molybdène, ou analogues, en une quantité de 20 à 50% en poids, de préférence d'environ 35% en poids, calculée par rapport au poids du fil sec de polyamides aromatiques comportant les particules solides.

13.- Corde, comme une corde marine, une corde de levage, et analogues, cette corde étant faite de deux ou plusieurs torons par pose ou tressage, caractérisée en ce que la corde est formée du fil selon la revendication 9.

14.- Procédé de fabrication du fil selon l'une quelconque des revendications 1 à 9, comprenant l'application au fil d'une dispersion de particules lubrifiantes solides de résines polyfluorocarbonées, en particulier de PTFE, et/ou de graphite, le fil étant soumis, à l'état humide, à un procédé d'entrelacement qui utilise un fluide sous pression, de préférence de l'air, à la suite de quoi les particules solides sont distribuées sur les filaments.

15.- Procédé selon la revendication 14, caractérisé en ce que le fluide est insufflé sur le fil dans la direction essentiellement transversale au mouvement du fil.

16.- Procédé selon la revendication 14, caractérisé en ce que l'on soumet le fil à un traitement de soufflage après lui avoir appliqué la dispersion contenant les particules solides.

17.- Procédé selon la revendication 14 ou 15, caractérisé en ce que la dispersion contenant des particules solides est appliquée au fil pendant le procédé de soufflage.

18.- Procédé selon la revendication 17, caractérisé en ce que la dispersion contenant des particules solides est appliquée directement aux filaments du fil par soufflage sur celui-ci sous pression.

19.- Procédé selon la revendication 14, caractérisé en ce que des particules solides chargées négativement d'une résine polyfluorocarbonée sont appliquées au fil à partir d'une dispersion aqueuse.

20.- Procédé selon la revendication 14, caractérisé en ce que des particules chargées positivement d'une résine polyfluorocarbonée sont appliquées au fil à partir d'une dispersion aqueuse.

21.- Procédé selon la revendication 19 ou 20, caractérisé en ce que la composition de la dispersion aqueuse est essentiellement la suivante:
- 45 à 75% en poids de particules de pTFE, de préférence environ 58% en poids;
- 50 à 20% en poids d'eau, de préférence environ 40% en poids;
- pas plus de 5% en poids d'un agent mouillant à base d'un alkylphénoxyéthanol, de préférence environ 3,5% en poids.

22.- Procédé selon la revendication 14, caractérisé en ce que l'excès de vitesse d'alimentation est d'au moins 1 %, de préférence d'environ 3% à 6%.
